

## UNITED STATES PATENT OFFICE

2,042,735

## METHOD OF AVOIDING COARSE CRYSTALLIZATION AT THE SOLIDIFICATION OF METALLIC CASTINGS

Erich Scheil, Dortmund, Germany, assignor to firm Vereinigte Stahlwerke Aktiengesellschaft, Dusseldorf, Germany

No Drawing. Application April 29, 1933, Serial No. 668,671. In Germany May 2, 1932

3 Claims. (Cl. 75—93)

Crystallization of a metal or alloy is known to proceed from single points called nuclei. During the solidification of the metal or alloy the number of these nuclei determines the size of the grain. The number of existing and spontaneously developing nuclei is so small in many alloys that a coarse grain is formed. The coarse grain reduces the capacity of the alloy for shaping without scraping or renders it even impossible and otherwise also injures the mechanical properties of alloys.

The measures generally employed against this coarseness of grain are accelerated cooling and low pouring temperature. The first measure is of course effective only at small cross sections of ingots. The effectiveness of the second measure does not suffice in all cases. Furthermore, the carrying out of this measure, particularly when casting large units, involves considerable difficulties.

According to the invention, coarseness of grain is reduced by artificially increasing the nuclei present in the liquid metal by additions, so that the structure of the ingot will become fine-grained and the working thereof by forging, rolling, drawing or similar deforming processes will be facilitated or made possible.

The production of these nuclei can, as a matter of principle, take place by means of various substances. Most effective is the addition of such kinds of crystals which are equal to those produced at the crystallization of the melt or isomorphous.

In the simplest way this increase of nuclei can be effected by the addition of solid pieces of the same alloy to the melt. Addition ought to take place after the finishing of the metallurgical operations, such as alloying, deoxidizing, degasifying, or the like. These pieces which might be referred to as generators of nuclei must dissolve in the melt to such an extent that after solidification substantially no unmelted parts can be noted, since that would cause defects in the casting. There will remain then in the melt very many much more difficultly destroyable nuclei which grow into crystals during solidification and thus produce a fine grain. The finer-grained the material of the nucleus generator the more nuclei will remain. Gradually, however, these nuclei will melt too, so that the number of nuclei will be the greater the shorter the time is between addition of the nucleus generator and solidification. If the melting speed of the nuclei of pieces of the same alloy is too great or if the time between the addition of the

nucleus generator and the solidification of the alloy, for any reasons, cannot be chosen short enough to attain a grain of sufficient fineness, the addition alloy may slightly deviate from the composition of the melt so as to have a higher melting point being approximately 50° C. above the melting point of the main alloy.

Harmful destruction of nuclei will be the smaller the lower the temperature of the melt is at the addition of the nucleus generator. From this, regulation of the pouring temperature can be derived without trouble. It should be as low as possible, though still high enough to insure perfect dissolution of the nucleus carriers. As a rule, a change of the normal casting temperature is unnecessary.

Any motion of the melt after the addition of the nucleus generator will have a destructive effect upon the nuclei also. Motions will be slightest when the nucleus generator is inserted into the mould (chill or sand mould) and molten only upon the pouring in of the liquid metal to be cast leaving the desired residual nuclei. For example, the nucleus generator may be secured in the mould in the form of a rod or wire. The number of rods and their thickness should be chosen so that the motion always occurring in the melt in the mould suffices for the uniform distribution of the nuclei, which should be ascertained by simple experiments as the case arises.

The invention may be applied for instance to steel or zinc melts in the following manner: 4 t. of a steel melt with 4% silicon were cast into a chill mould of a bar cross-section of 500 x 500 mm., 10 bars of the nuclei generator having a thickness of 5—20 mm. were distributed over this cross-section. The bars may for instance be put into the mould in a vertical position and secured at the bottom and the top of the mould by means of iron plates. In this manner a very fine grain could be obtained. With zinc melts which have a great tendency to transcrystallization, it was possible almost completely to obviate said transcrystallization by inserting 4 wires of a thickness of 1 mm. into a 20 kg. melt which was cast into a round chill mould of a bar cross-section of 100 mm<sup>2</sup>.

In the neighbourhood of the cooling wall the thickness of the rods should probably be chosen somewhat less. The thickness of the rods of the nucleus generator should be adapted to the wall thickness of the ingot in such a way that it will be the greater the greater the cross section of the ingot, since otherwise the nucleus generators would be destroyed too quickly and,

at the long solidification period, a large number of the residual nuclei would be destroyed also.

With this arrangement of the nucleus generator quick cooling from the sides by a chill mould usually employed in case of forging ingots 5 may be dispensed with and in lieu thereof a sand mould used. Thus internal stresses which are quite large in quickly solidified large ingots will be very much reduced.

10 The amount of material added as nucleus generator differs and can be stated only approximately; the lower limit of effectiveness will be approximately near 0.1% of the casting. However, the amount of nucleus material may be 15 much higher and, for instance, be as high as about 5%.

If the material of the nucleus generator corrodes easily or forms scale to a considerable degree during heating, so that at contact with 20 the melt gases or at least flaws develop, it may be provided with a protective covering of a known kind protecting the inserted rods or the like against corrosion and scaling.

Instead of arranging the nucleus generator in 25 the mould, it may be added by throwing small pieces thereof into the casting jet.

Both methods, that is, arrangement of the nucleus generator in the mould and throwing it into the jet or addition to the ladle, may be 30 combined. It will then be advantageous to increase the addition to the jet towards the end of the casting operation. It is further advisable to provide for a larger diameter on top of the ingot than below in order to avoid piping.

35 In the foregoing it has been stated that the nucleus generators are to be added in the form of pieces which are adapted to be substantially destroyed by the available heat, that is, to such an extent that only small yet numerous remnants are left in the melt. Said remnants will be of microscopic or sub-microscopic size which 40 is sufficient for forming nuclei. The exact shape and dimensions of the inserted substances which are suitable for each purpose can easily be determined in practice by a simple test. For this purpose preliminary test bars of different thickness are inserted and the variation in thickness is continued until the microscopic inspection shows a complete or a nearly complete melting of the 45

added substance, so that the nucleus generator is present only in microscopic or sub-microscopic parts.

What I claim and desire to secure by Letters Patent in the United States is:

1. Method of obtaining a fine crystallization of metallic castings in order to enhance their workability which consists in adding to the liquid metal several solid pieces of the same alloy as the cast material, the size of said pieces being 10 determined in accordance with the transcrystallization tendency of the metal in such a manner that they are completely molten before the casting ingots begin to solidify, but leaving numerous very small invisible remnants forming nuclei 15 during the solidification of the ingots.

2. Method of obtaining a fine crystallization of metallic castings in order to enhance their workability which consists in adding to the liquid metal several solid pieces of a metal or metal 20 alloy of an isomorphous crystalline structure having a melting point up to 50° C. higher than the metal to be cast, the size of said pieces being determined in accordance with the transcrystallization tendency of the metal in such a manner 25 that they are completely molten before the casting ingots begin to solidify, but leaving numerous very small invisible remnants forming nuclei during the solidification of the ingots.

3. Method of obtaining a fine crystallization of 30 metallic castings in order to enhance their workability which consists in inserting into the mould several barlike solid pieces of a metal or metal alloy of a fine grained material and of a structure at least isomorphous to that of the metal to 35 be cast, the size of said pieces being adapted to the transcrystallization tendency of the metal to be cast in such a manner that they are completely molten before the casting ingots begin to solidify and securing them therein prior to the 40 casting operation, thereupon pouring in the metal to be cast, thereby melting the inserted pieces from the bottom upwards in accordance with the rise in level of the liquid to such an extent that only numerous very small invisible 45 remnants are left in the melt of a size sufficient for forming nuclei during the solidification of the ingots.

ERICH SCHEIL.